# EUROPEAN PATENT SPECIFICATION

(11) **EP 1 959 773 B1**
(45) Date of publication and mention of the grant of the patent: **11.11.2009**
(21) Application number: 06846588.9
(22) Date of filing: 13.12.2006
(51) Int. Cl.: A41D 31/00, D02G 3/44

(54) **THERMAL PERFORMANCE GARMENTS COMPRISING AN OUTER SHELL FABRIC OF PIPD AND ARAMID FIBERS**
WÄRMELEISTUNGSKLEIDUNGSSTÜCKE MIT EINEM AUSSENHAUTSTOFF AUS PIPD- UND ARAMIDFASERN
VÊTEMENTS PRÉSENTANT DES PROPRIÉTÉS THERMIQUES COMPOSÉS D'UN TISSU DE REVÊTEMENT EXTÉRIEUR COMPRENANT DES FIBRES PIPD ET ARAMIDES

(30) Priority: 16.12.2005 US 751151 P
(43) Date of publication of application: 27.08.2008
(73) Proprietor: E.I. DU PONT DE NEMOURS AND COMPANY, Wilmington, DE 19898 (US)
(72) Inventor: ZHU, Reiyao H., Midlothian, Virginia 23112 (US); YOUNG, Richard, Richmond, Virginia 23236 (US)
(74) Representative: Heinemann, Monica
(86) International application number: PCT/US2006/061985
(87) International publication number: WO 2007/073539

(56) References cited:
- EP-A1- 1 386 987
- WO-A1-99/27169
- US-A- 4 865 906
- US-A1- 2004 034 905

## Description

### FIELD OF THE INVENTION

The invention concerns a flame-resistant garment having an outer shell fabric comprising polypyridobisimidazole fiber and aramid fiber.

### BACKGROUND OF THE INVENTION

Polypyridobisimidazole polymer is a rigid rod polymer. Fiber made from this polymer, one polymer composition of which is referred to as PIPD and known as the polymer used to make M5® fiber, is known to be useful in both cut and flame resistant protective apparel. See, for example, PCT Application WO19990216 and WO2005002376. Fibers made from rigid-rod polymers having strong hydrogen bonds between polymer chains, e.g., polypyridobisimidazoles, have been described in U.S. Pat. No. 5,674,969 to Sikkema et al. An example of a polypyridobisimidazole includes poly(1,4-(2,5-dihydroxy)phenylene-2,6-pyrido[2,3-d:5,6-d']bisimidazole), which can be prepared by the condensation polymerization of tetraaminopyridine and 2,5-dihydroxyterephthalic acid in polyphosphoric acid. Sikkema describes that in making one- or two-dimensional objects, such as fibers, films, tapes, and the like, it is desired that polypyridobisimidazoles have a high molecular weight corresponding to a relative viscosity ("Vᵣₑₗ" or "ηᵣₑₗ") of at least about 3.5, preferably at least about 5, and more particularly equal to or higher than about 10, when measured at a polymer concentration of 0.25 g/dl in methane sulfonic acid at 25°C. Sikkema also discloses that good fiber spinning results are obtained with poly[pyridobisimidazole-2,6-diyl(2,5-dihydroxy-p-phenylene)] having relative viscosities greater than about 12, and that relative viscosities of over 50 (corresponding to inherent viscosities greater than about 15.6 dl/g) can be achieved.

Published U.S. Patent Applications US20030228812, US20040216215 and US20040034905 and U.S. Patent No. 6,624,096 disclose protective fabrics & garments made from blends of Kevlat® and polybenzimidazole (PBI).

The aforementioned polybenzimidazoles are polybibenzimidazole compositions, which are not rigid rod polymers. Therefore the fiber made from that polymer has low fiber strength.

Thermal and flame retardant protective apparel has been used by firefighters, emergency response personnel, members of the military and racing personnel, as well as industrial workers to save lives and reduce injury due to fires and other thermal events. While polypyridobisimidazole fiber has excellent fire resistant properties, superior in many respects to most other fibers, it also has a very high tensile modulus or modulus of elasticity. One concern with using such fibers is that they have a high modulus and may create fabrics that are relatively stiff and uncomfortable to wear. There is, however, a desire to incorporate the superior fire resistance of polypyridobisimidazole fibers into fabrics to take advantage of their superior flame resistant properties. Thus, there is a need for a fabric containing polypyridobisimidazole that is both comfortable and still provides good fire protective performace.

### SUMMARY OF THE INVENTION

In some embodiments, the invention concerns flame-resistant garment comprising polypyridobisimidazole fiber and aramid fiber. In certain embodiments, the invention concerns a flame-resistant garment comprising 30 to 70 parts by weight of a polypyridobisimidazole fiber and 70 to 30 parts by weight of an aramid fiber; the polypyridobisimidazole fiber having an inherent viscosity of greater than 20 dl/g. In some embodiments, the polypyridobisimidazole fiber has an inherent viscosity of greater than 25 dl/g. In other embodiments, the polypyridobisimidazole fiber has an inherent viscosity of greater than 28 dl/g

Some flame-resistant garments of this invention comprise 40 to 60 parts by weight of a polypyridobisimidazole fiber, and 60 to 40 parts by weight of an aramid fiber.

In some embodiments, the polypyridobisirnidazole and aramid fibers are present as staple fibers. In certain embodiments, the polypyridobisimidazole and aramid fibers are present as continuous filaments.

One preferred polypyridobisimidazole polymer is poly[2,6-diimidazo[4,5-b:4,5-e]- pyridinylene-1,4(2,5-dihydroxy)phenylene).

Some preferred aramid fiber comprises para-aramid polymer. Poly(paraphenylene terephthalamide) is one preferred para-aramid polymer.

In some embodiments, the polypyridobisimidazole and aramid fibers are in the outer shell of the garment.

In another aspect, the invention concerns a flame-resistant garment comprising, in order, (a) an inner thermal lining, (b) a liquid barrier, and (c) an outer shell fabric, the outer shell fabric (c) comprising 30 to 70 parts by weight of a polypyridobisimidazole fiber and 30 to 70 parts by weight of an aramid fiber; the polypyridobisimidazole fiber having an inherent viscosity of greater than 20 dl/g.

Additional embodiments of the invention concern method of producing a flame-resistant garment having an inner thermal lining, a liquid barrier, and an outer shell fabric by incorporating into the garment an outer shell fabric comprising 30 to 70 parts by weight of a polypyridobisimidazole fiber and 70 to 30 parts by weight of an aramid fiber; the polypyridobisimidazole fiber having an inherent viscosity of greater than 20 dl/g.

### DETAILED DESCRIPTION OF ILLUSTRATIVE EMBODIMENTS

The present invention may be understood more readily by reference to the following detailed description of illustrative and preferred embodiments that form a part of this disclosure. It is to be understood that the scope of the claims is not limited to the specific devices, methods, conditions or parameters described and/or shown herein, and that the terminology used herein is for the purpose of describing particular embodiments by way of example only and is not intended to be limiting of the claimed invention. Also, as used in the specification including the appended claims, the singular forms "a," "an," and "the" include the plural, and reference to a particular numerical value includes at least that particular value, unless the context clearly dictates otherwise. When a range of values is expressed, another embodiment includes from the one particular value and/or to the other particular value. Similarly, when values are expressed as approximations, by use of the antecedent "about," it will be understood that the particular value forms another embodiment. All ranges are inclusive and combinable.

In one embodiment, the invention relates to a flame-resistant garment having an outer shell fabric comprising 30 to 70 parts by weight of a polypyridobisimidazole fiber and 30 to 70 parts by weight of an aramid fiber, the polypyridobisimidazole fiber having an inherent viscosity of greater than 20 dl/g. This invention also relates to a flame-resistant garment comprising, in order, an inner thermal lining, a liquid barrier, and an outer shell fabric; the outer shell fabric comprising 30 to 70 parts by weight of a polypyridobisimidazole fiber and 30 to 70 parts by weight of an aramid fiber and the polypyridobisimidazole fiber having an inherent viscosity of greater than 20 dl/g.

For purposes herein, the term "fiber" is defined as a relatively flexible, macroscopically homogeneous body having a high ratio of length to width across its cross-sectional area perpendicular to its length. The fiber cross section can be any shape, but is typically round. Herein, the term "filament" or "continuous filament" is used interchangeably with the term "fiber."

As used herein, the term "staple fibers" refers to fibers that are cut to a desired length or are stretch broken, or fibers that occur naturally with or naturally have a low ratio of length to width across its cross-sectional area perpendicular to its length when compared with filaments. Length can vary from about 0.1 inch to several feet. In some embodiments, the length is from 0.1 inch to about 8 inches. Man made staple fibers are cut to a length suitable for processing on cotton, woolen, or worsted yarn spinning equipment.

The staple fibers can have (a) substantially uniform length, (b) variable or random length, or (c) subsets of the staple fibers have substantially uniform length and the staple fibers in the other subsets have different lengths, with the staple fibers in the subsets mixed together forming a substantially uniform distribution.

In some embodiments, suitable staple fibers have a length of 1 to 30 centimeters. Staple fibers made by short staple processes result in a fiber length of 1 to 6 centimeters.

The staple fibers can be made by any process. The staple fibers can formed by stretch breaking continuous fibers resulting in staple fibers with deformed sections that act as crimps. The staple fibers can be cut from continuous straight fibers using a rotary cutter or a guillotine cutter resulting in straight (i.e., non crimped) staple fiber, or additionally cut from crimped continuous fibers having a saw tooth shaped crimp along the length of the staple fiber, with a crimp (or repeating bend) frequency of no more than 8 crimps per centimeter.

Stretch broken staple fibers can be made by breaking a tow or a bundle of continuous filaments during a stretch break operation having one or more break zones that are a prescribed distance creating a random variable mass of fibers having an average cut length controlled by break zone adjustment.

Staple fibers of this invention can be converted into yarns using traditional long and short staple ring spinning processes which are well known in the art. For short staple, cotton system spinning fiber lengths from 3/4 inch to 2-1/4 inch (i.e., 1.9 to 5.7 cm.) are typically used. For long staple, worsted or woolen system spinning, fibers up to 6-1/2 inches (i.e., 16.5 cm.) are typically used. However, this is not intended to be limiting to ring spinning because the yarns may also be spun using air jet spinning, open end spinning, and many other types of spinning which converts staple fiber into useable yarns.

The stretch broken staple fibers typically have length of up to 7 inches (i.e., 17.8 cm.) long and can be made using traditional stretch-broken tow to top staple processes. Staple fibers having maximum lengths of up to around 20 inches (i.e., 51 cm) are possible through processes as described for example in PCT Patent Application No. WO 0077283. Yarns can be made by consolidating fibers into spun yarn using filament entanglement with air jets having a tenacity in the range of 3 to 7 grams per decitex. These yarns may have secondary twist, that is, they may be twisted after formation to impart more tenacity to the yam, in which case the tenacity can be in the 10 to 18 grams per denier (i.e., 9 to 17 grams per dtex) range. Stretch broken staple fibers normally do not require crimp because the stretch-breaking process imparts a degree of crimp into the fiber.

The term continuous filament refers to a flexible fiber having relatively small-diameter and whose length is longer than those indicated for staple fibers. Continuous filament fibers and multifilament yarns of continuous filaments can be made by processes well known to those skilled in the art.

Fabrics of this invention can take on numerous configurations, including, but not limited to, knitted or woven fabrics or non-woven structures. Such fabric configurations are well known to those skilled in the art.

By "non-woven" fabric is meant a network of fibers, including unidirectional (if contained within a matrix resin), felt, fiber batts, and the like.

By "woven" fabric is meant a fabric woven using any fabric weave, such as plain weave, crowfoot weave, basket weave, satin weave, twill weave, and the like. Plain and twill weaves arc believed to be the most common weaves used in the trade.

The instant invention utilizes polypyridobisimidazole fiber. This fiber is a rigid rod polymer that is of high strength. The polypyridobisimidazole fiber has an inherent viscosity of at least 20 dl/g or at least 25 dl/g or at least 28 dl/g. Such fibers include PIPD fiber (also known as M5® fiber and fiber made from poly[2,6-diimidazo[4,5-b:4,5-e]- pyridinylene-1,4(2,5-dihydroxy)phenylene). PTPD fiber is based on the structure:

Polypyridobisimidazole fiber can be distinguished from the well known commercially available PBI fiber or polybenzimidazole fiber in that that polybenzimidazole fiber is a polybibenzimidazole. Polybibenzimidazole fiber is not a rigid rod polymer and has low fiber strength and low tensile modulus when compared to polypyridobisimidazoles.

PIPD fibers have been reported to have the potential to have an average modulus of about 310 GPa (2100 grams/denier) and an average tenacities of up to about 5.8 Gpa (39.6 grams/denier). These fibers have been described by Brew, et al., Composites Science and Technology 1999, 59, 1109; Van der Jagt and Beukers, Polymer 1999, 40, 1035; Sikkema, Polymer 1998, 39, 5981; Klop and Lammers, Polymer, 1998, 39, 5987; Hagernan, et al., Polymer 1999, 40, 1313.

One method of making rigid rod polypyridoimidazole polymer is disclosed in detail in United States Patent 5,674,969 to Sikkema *et al.* Polypyridoimidazole polymer may be made by reacting a mix of dry ingredients with a polyphosphoric acid (PPA) solution. The dry ingredients may comprise pyridobisimidazole-forming monomers and metal powders. The polypyridobisimidazole polymer used to make the rigid rod fibers used in the fabrics of this invention should have at least 25 and preferably at least 100 repetitive units.

For the purposes of this invention, the relative molecular weights of the polypyridoimidazole polymers are suitably characterized by diluting the polymer products with a suitable solvent, such as methane sulfonic acid, to a polymer concentration of 0.05 g/dl, and measuring one or more dilute solution viscosity values at 30°C. Molecular weight development of polypyridoimidazole polymers of the present invention is suitably monitored by, and correlated to, one or more dilute solution viscosity measurements. Accordingly, dilute solution measurements of the relative viscosity ("Vᵣₑₗ" or "ηᵣₑₗ" or "nᵣₑₗ") and inherent viscosity ("Vᵢₙₕ" or "ηᵢₙₕ" or "nᵢₙₕ") are typically used for monitoring polymer molecular weight. The relative and inherent viscosities of dilute polymer solutions are related according to the expression ${V}_{inh} = ln \left({V}_{rel}\right) / C ,$
where *ln* is the natural logarithm function and C is the concentration of the polymer solution. Vᵣₑₗ is a unitlcss ratio of the polymer solution viscosity to that of the solvent free of polymer, thus Vᵢₙₕ is expressed in units of inverse concentration, typically as deciliters per gram ("dl/g"). Accordingly, in certain aspects of the present invention the polypyridoimidazole polymers are produced that are characterized as providing a polymer solution having an inherent viscosity of at least about 20 dl/g at 30°C at a polymer concentration of 0.05 g/dl in methane sulfonic acid. Because the higher molecular weight polymers that result from the invention disclosed herein give rise to viscous polymer solutions, a concentration of about 0.05 g/dl polymer in methane sulfonic acid is useful for measuring inherent viscosities in a reasonable amount of time.

Exemplary pyridobisimidazole-forming monomers useful in this invention include 2,3,5,6-tetraaminopyridine and a variety of acids, including terephthalic acid, bis-(4-benzoic acid), oxy-bis-(4-benzoic acid), 2,5-dihydroxyterephthalic acid, isophthalic acid, 2,5-pyridodicarboxylic acid, 2,6-napthalenedicarboxylic acid, 2,6-quinolinedicarboxylic acid, or any combination thereof. Preferably, the pyridobisimidazole forming monomers include 2,3,5,6-tetraaminopyridine and 2,5-dihydroxyterephthalic acid. In certain embodiments, it is preferred that that the pyridoimidazole-forming monomers are phosphorylated. Preferably, phosphorylated pyridoimidazole-forming monomers are polymerized in the presence of polyphosphoric acid and a metal catalyst.

Metal powders can be employed to help build the molecular weight of the final polymer. The metal powders typically include iron powder, tin powder, vanadium powder, chromium powder, and any combination thereof.

The pyridobisimidazole-forming monomers and metal powders are mixed and then the mixture is reacted with polyphosphoric acid to form a polypyridoimidazole polymer solution. Additional polyphosphoric acid can be added to the polymer solution if desired. The polymer solution is typically extruded or spun through a die or spinneret to prepare or spin filaments.

By "aramid" is meant a polyamide wherein at least 85% of the amide (-CO-NH-) linkages are attached directly to two aromatic rings. Suitable aramid fibers are described in Man-Made Fibers - Science and Technology, Volume 2, Section titled Fiber-Forming Aromatic Polyamides, page 297, W. Black et al., Interscience Publishers, 1968.
Aramid fibers are, also, disclosed in U.S. Patent Nos. 4,172,938; 3,869,429; 3,819,587; 3,673,143; 3,354,127; and 3,094,511. Additives can be used with the aramid and it has been found that up to as much as 10 percent, by weight, of other polymeric material can be blended with the aramid or that copolymers can be used having as much as 10 percent of other diamine substituted for the diamine of the aramid or as much as 10 percent of other diacid chloride substituted for the diacid chloride or the aramid.

One preferred aramid is a para-aramid and poly(p-phenylene terephthalamide)(PPD-T) is the preferred para-aramid. By PPD-T is meant the homopolymer resulting from approximately mole-for-mole polymerization of p-phenylene diamine and terephthaloyl chloride and, also, copolymers resulting from incorporation of small amounts of other diamines with the p-phenylene diamine and of small amounts of other diacid chlorides with the terephthaloyl chloride. As a general rule, other diamines and other diacid chlorides can be used in amounts up to as much as about 10 mole percent of the p-phenylene diamine or the terephthaloyl chloride, or perhaps slightly higher, provided only that the other diamines and diacid chlorides have no reactive groups which interfere with the polymerization reaction. PPD-T, also, means copolymers resulting from incorporation of other aromatic diamines and other aromatic diacid chlorides such as, for example, 2,6-naphthaloyl chloride or chloro- or dichloroterephthaloyl chloride or 3,4'-diaminodiphenylether. One suitable para-aramid is sold by E.I. du Pont de Nemours and Company under the tradename KEVLAR®. In some embodiments, the aramid can be meta-aramid and poly(m-phenylene isophthalamide) is the preferred meta-aramid. One suitable meta-aramid is sold by E.I. du Pont de Nemours and Company under the trademark NOMEX®.

As illustration of some particularly useful embodiments of this invention, the flame-resistant garment can have essentially one layer, which is the outer shell fabric, for such things as jumpsuits for fire fighters or for military personnel. Such suits are typically used over the firefighters clothing and can be used to parachute into an area to fight a forest fire.

In other embodiments of this invention the flame-resistant garment is as multilayer garment having a general construction such as disclosed in United States Patent No. 5,468,537, which is incorporated by reference. Such garments generally have three layers or three types of fabric constructions, each layer or fabric construction performing a distinct function. There is an outer shell fabric that provides flame protection and serves as a primary defense from flames for the fire fighter. Adjacent the outer shell is a moisture barrier that is typically a liquid barrier but can be selected such that it allows moisture vapor to past through the barrier. Laminates of Gore-Tex® PTFE membrane or Neoprene® membranes on a fibrous nonwoven or woven meta-aramid scrim fabric are moisture barriers typically used in such constructions. Adjacent the moisture barrier is a thermal liner, which generally includes a batt of heat resistant fiber attached to an internal face cloth. The moisture barrier keeps the thermal liner dry and thermal liner protects the wearer from heat stress from the fire or heat threat being addressed by the wearer.

The outer shell fabric of the garments of this invention have 30 to 70 parts by weight of a polypyridobisimidazole fiber and 30 to 70 parts by weight of an aramid fiber, based on 100 parts by weight of the two fibers. This compositional range is believed to provide the best combination of properties from both fibers with the high performance and high cost of the polypyridobisimidazole fiber being combined with the lower modulus and lower cost of the aramid fiber to provide a garment fabric that is both durable, high performance, and yet can be provided with a reasonable cost. In some preferred embodiments, the compositional range of the outer shell fabric of the garments of this invention have 40 to 60 parts by weight of a polypyridobisimidazole fiber and 40 to 60 parts by weight of an aramid fiber, based on 100 parts by weight of the two fibers.

The garments of this invention have improved outer fabrics. Polypyridobisimidazole yarns typically have a very high tensile modulus, which is generally about 600 to 2300 grams per denier. In some preferred embodiments for apparel, the tensile modulus is 1000 to 1800 grams per denier. A yarn having a high tensile modulus translates, in many cases, to a stiffer fabric, so a fabric made totally from polypyridobisimidazole yarns would reflect the high tensile modulus of the fiber. In some preferred embodiments the aramid fiber is polyparaphenylene terephthalamide, and fibers of this type that have use in apparel have a tensile modulus of about 400 to 900 grams per denier, preferably 400 to 600 grams per denier. In other embodiments the aramid fiber is polymetaphenylene isophthalamide, and fibers of this type have a tensile modulus of less than about 100 grams per denier, typically about 50 to 90 grams per denier. Therefore, in the most preferred embodiments the aramid fiber has a tensile modulus that is less that the tensile modulus of the polypyridobisimidazole fiber. This ensures that the fabric will generally have lower stiffness than therefore more flexible than a fabric made totally from the high modulus polypyridobisimidazole fiber.

When the aramid fiber used with the polypyridobisimidazole fiber in the outer fabric is a high toughness fiber such as the polyparaphenylene terephthalamide fiber, the combination with high strength polypyridobisimidazole fiber will ensure the resulting flame-retardant fabric has higher-strength than the prior art outer fabrics that are made form the combination of polyparaphenylene terephthalamide and polybibenzimidazole fibers. When the aramid used with the polypyridobisimidazole fiber in the outer fabric is a lower modulus aramid fiber such as polymetaphenylene isophthalamide, the combination with the polypyridobisimidazole fiber will ensure the resulting fabrtic is very flexible and has advanced flame retardant properties.

In a preferred embodiment of this invention the outer shell fabric is woven. The fibers can be incorporated into the outer shell fabric using staple fibers yarns of an intimate blend of fibers. By "intimate blend", it is meant the various staple fibers in the blend form a relatively uniform mixture of the fibers. If desired, other staple fibers can be combined in this relatively uniform mixture of staple fibers. The blending can be achieved by any number of ways known in the art, including processes that creel a number of bobbins of continuous filaments and concurrently cut the two or more types of filaments to form a blend of cut staple fibers; or processes that involve opening bales of different staple fibers and then opening and blending the various fibers in openers, blenders, and cards; or processes that form slivers of various staple fibers which are then further processed to form a mixture, such as in a card to form a sliver of a mixture of fibers. Other processes of making an intimate fiber blend are possible as long as the various types of different fibers are relatively uniformly distributed throughout the blend. If yarns are formed from the blend, the yarns have a relatively uniform mixture of the staple fibers also. Generally, in most preferred embodiments the individual staple fibers are opened or separated to a degree that is normal in fiber processing to make a useful fabric, such that fiber knots or slubs and other major defects due to poor opening of the staple fibers are not present in an amount that detract from the final fabric quality.

Alternatively, some woven fabrics of this invention can be made by weaving individual ends of polypyridobisimidazole fiber staple yarns with individual ends of aramid fiber staple yarns. This can be achieved in any number of ways, such as plying the two different staple yarns together or by weaving a portion of one type of staple fiber in the warp and another type of staple fiber in the fill.

Alternatively, some woven fabrics of this invention can be made from multifilament continuous yarns which are either a mixture of different filaments, or as indicated above for different staple yarns, arc woven from individual ends of different multifilament yarns.

This invention also relates to a method of producing a flame-resistant garment having an inner thermal lining, a liquid barrier, and an outer shell fabric by incorporating into the garment an outer shell fabric comprising 30 to 70 parts by weight of a polypyridobisimidazole fiber and 70 to 30 parts by weight of an aramid fiber; the polypyridobisimidazole fiber having an inherent viscosity of greater than 20 dl/g. In some preferred embodiments, the polypyridobisimidazole fiber comprises poly[2,6-diimidazo[4,5-b:4,5-e]- pyridinylene-1,4(2,5-dihydroxy)phenylene) and the aramid fiber comprises poly(paraphenylene terephthalamide).

### Test Methods

**Thermal Protective Performance Test (TPP). The predicted protective** performance of a fabric in heat and flame is measured using the "Thermal Protective Performance Test" NFPA 2112 (referred to as "TPP"). A flame is directed at a section of fabric mounted in a horizontal position at a specified heat flux (typically 84 kW/m²). The test measures the transmitted heat energy from the source through the specimen using a copper slug calorimeter with no space between the fabric and heat source. The test endpoint is characterized by the time required to attain a predicted second-degree skin burn injury using a simplified model developed by Stoll & Chianta, "Transactions New York Academy Science", 1971, 33 p 649. The value assigned to a specimen in this test, denoted as the TPP value, is the total heat energy required to attain the endpoint, or the direct heat source exposure time to the predicted burn injury multiplied by the incident heat flux. Higher TPP values denote better insulation performance.

### Examples

The invention is illustrated by, but is not intended to be limited by the following examples.

### Example 1

A thermally protective and durable fabric is prepared having in both the warp and fill ring spun yarns of intimate blends of para-aramid fiber, polypyridobisimidazole staple fiber, and antistatic staple fiber. The para-aramid staple fiber is made from poly(p-phenylene terephthalamide)(PPD-T) polymer and is marketed by DuPont under the trademark Kevlar® 29 fiber, the polypyridobisimidazole staple fiber is made from PIPD polymer and is marketed by Magellan Systems International under the trademark M5® fiber, and the antistatic staple fiber has a nylon sheath and carbon core and is known as P-140 nylon fiber, available from Invista.

A picker blend sliver of 38 wt.% of polypyridobisimidazole, 60% of para-aramid, and 2 wt. % of antistatic fiber is prepared and processed by the conventional cotton system equipment and is then spun into a spun staple yarn having twist multiplier 4.0 and a single yarn size of about 21 tex (28 cotton count) using a ring spinning frame. Two single yarns are then plied on a plying machine to make a two-ply yarn. Using a similar process and the same twist and blend ratio, a 24 tex (24 cotton count) yarn is made for use as a fill yarn. As before, two of these single yarns are plied to form a two-ply yarn.

The para-aramid/polypyridobisimidazole/antistatic yarns blend yarns are then used as the warp and fill yarns and are woven into a fabric on a shuttle loom, making a greige fabric having a 2x1 twill weave and a construction of 26 ends x 17 picks per cm (72 ends x 52 picks per inch), and a basis weight of about 215 g/m² (6.5 oz/yd²). The greige twill fabric is then scoured in hot water and is dried under low tension. The scoured fabric is then jet dyed using basic dye. The finished fabric has a basis weight of about 231 g/m² (7 oz/yd²).

The finished fabric is then used as an outershell fabric for a three-layer composite fabric that also includes a moisture barrier and a thermal liner. The moisture barrier is Goretex (0.5-0.8oz/yd2) with a nonwoven MPD-I/PPD-T fiber substrate (2.7oz/yd2) and thermal liner is three spunlaced l.Soz/yd2 sheets quilted to a 3.2oz/yd2 MPD-1 staple fiber scrim. A sample of the composite fabric, when exposed to flame in the Thermal Protective Performance Test (TPP) has high TTP values.

### Example 2

Alternatively, the finished fabric of Example 1 is made into protective articles, including garments, by cutting the fabric into fabric shapes per a pattern and sewing the shapes together to form a protective coverall for use as protective apparel in industry. Likewise, the fabric is cut into fabric shapes and the shapes sewn together to form a protective apparel combination comprising a protective shirt and a pair of protective pants. If desired, the fabric is cut and sewn to form other protective apparel components such as hoods, sleeves, and aprons.

### Example 3

A fabric containing 60% by weight para-aramid staple fiber made from poly(p-phenylene terephthatamide)(PPD-T) polymer and marketed by DuPont under the trademark Kevlar® 29 fiber, and 40% polypyridobisimidazole staple fiber made from PIPD polymer and marketed by Magellan Systems International under the trademark M5® fiber was made as disclosed in Example 1, however, this fabrics did not contain any antistatic fiber. The fabric had a basis weight of about 242 g/m² (7.14 oz/yd²) and the time required to attain a predicted second-degree skin burn injury using the TPP test was 7.03 sec using an incident heat flux of 2 calories/cm²/sec. The calculated TPP value (energy) was 14.06 calories/cm².

### Example 4

Example 3 was repeated, however the 60% by weight PPD-T fiber was replaced with meta-aramid staple fiber made from poly(m-phenylene isophthatamide)(WD-I) polymer and marketed by DuPont under the trademark Nomex® fiber, The fabric had a basis weight of about 260 g/m² (7.68 oz/yd²) and the time required to attain a predicted second-degree skin burn injury using the TPP test was 7.01 sec using an incident heat flux of 2 calories/cm²/ sec. The calculated TPP value (energy) was 14.02 calories/cm².

## Claims

1. A flame-resistant garment having an outer shell fabric comprising:
30 to 70 parts by weight of a polypyridobisimidazole fiber having an inherent viscosity of greater than 20 dl/g and
30 to 70 parts by weight of an aramid fiber.

2. The flame-resistant garment of claim 1 where the polypyridobisimidazole fiber has an inherent viscosity of greater than 25 dl/g, preferably of greater than 28 dl/g.

3. The flame-resistant garment of claim 1 comprising
40 to 60 parts by weight of a polypyridobisimidazole fiber, and
40 to 60 parts by weight of an aramid fiber.

4. The flame-resistant garment of claim 1 where the polypyridobisimidazole or aramid fibers are present as staple fibers, and where the polypyridobisimidazole preferably is poly[2,6-diimidazo[4,5-b:4,5-e]- pyridinylene-1,4(2,5-dihydroxy)phenylene).

5. The flame-resistant garment of claim 1 wherein the aramid fibers are para-aramid fibers, and where the para-aramid fiber preferably comprises poly(paraphenylene terephthalamide) polymer.

6. The flame-resistant garment of claim 1 where the polypyridobisimidazole or aramid fibers are present as continuous filaments.

7. A flame-resistant garment comprising in order
a) an inner thermal lining,
b) a liquid barrier, and
c) an outer shell fabric,
the outer shell fabric comprising:
30 to 70 parts by weight of a polypyridobisimidazole fiber having an inherent viscosity of greater than 20 dl/g and
30 to 70 parts by weight of an aramid fiber.

8. The flame-resistant garment of claim 7 where the polypyridobisimidazole fiber has an inherent viscosity of greater than 25 dl/g, preferably of greater than 28 dl/g.

9. The flame-resistant garment of claim 7 where the outer shell fabric comprises:
40 to 60 parts by weight of a polypyridobisimidazole fiber, and
40 to 60 parts by weight of an aramid fiber.

10. The flame-resistant garment of claim 7 where the polypyridobisimidazole or aramid fibers are present as staple fibers, and where the polypyrimidazole polymer preferably is poly[2,6-diimidazo[4,5-b:4,5-c]- pyridinylene-1,4(2,5-dihydroxy)phenylene).

11. The flame-resistant garment of claim 7 wherein the aramid fibers are para-aramid fibers, and where the para-aramid fiber preferably comprises poly(paraphenylene terephthalamide) polymer.

12. The flame-resistant garment of claim 7 where the polypyridobisimidazole or aramid fibers are present as continuous filaments.

13. A method of producing a flame-resistant garment having an inner thermal lining, a liquid barrier, and an outer shell fabric, by incorporating into the garment an outer shell fabric comprising
40 to 60 parts by weight of a polypyridobisimidazole fiber, and
40 to 60 parts by weight of an aramid fiber.

14. The method of claim 13 where the polypyridobisimidazole fiber comprises poly[2,6-diimidazo[4,5-b:4,5-e]- pyridinylene-1,4(2,5-dihydroxy)phenylene) and the aramid fiber comprises poly(paraphenylene terephthalamide).

## Patentansprüche

1. Flammbeständiges Kleidungsstück mit einem Außenhautgewebe, das aufweist:
30 bis 70 Gewichtsteile einer Polypyridobisimidazol-Faser mit einer Eigenviskosität von mehr als 20 dl/g und
30 bis 70 Gewichtsteile einer Aramidfaser.

2. Flammbeständiges Kleidungsstück nach Anspruch 1, wobei die Polypyridobisimidazol-Faser eine Eigenviskosität von mehr als 25 dl/g, vorzugsweise von mehr als 28 dl/g aufweist.

3. Flammbeständiges Kleidungsstück nach Anspruch 1, das aufweist:
40 bis 60 Gewichtsteile einer Polypyridobisimidazol-Faser, und
40 bis 60 Gewichtsteile einer Aramidfaser.

4. Flammbeständiges Kleidungsstück nach Anspruch 1, wobei die Polypyridobisimidazol- oder Aramidfasern als Stapelfasern anwesend sind, und wobei das Polypyridobisimidazol vorzugsweise Poly[2,6-diimidazo[4,5-b:4,5-e]pyridinylen-1,4-(2,5-dihydroxy)phenylen] ist.

5. Flammbeständiges Kleidungsstück nach Anspruch 1, wobei die Aramidfasern para-Aramidfasern sind, und wobei die para-Aramidfaser vorzugsweise Poly(paraphenylenterephtalamid)-Polymer aufweist.

6. Flammbeständiges Kleidungsstück nach Anspruch 1, wobei die Polypyridobisimidazol- oder Aramidfasern als Endlosfilamente anwesend sind.

7. Flammbeständiges Kleidungsstück, das in dieser Reihenfolge aufweist:
a) ein inneres Thermofutter,
b) eine Flüssigkeitssperrschicht, und
c) ein Außenhautgewebe,
wobei das Außenhautgewebe aufweist:
30 bis 70 Gewichtsteile einer Polypyridobisimidazol-Faser mit einer Eigenviskosität von mehr als 20 dl/g und
30 bis 70 Gewichtsteile einer Aramidfaser.

8. Flammbeständiges Kleidungsstück nach Anspruch 7, wobei die Polypyridobisimidazol-Faser eine Eigenviskosität von mehr als 25 dl/g, vorzugsweise von mehr als 28 dl/g aufweist.

9. Flammbeständiges Kleidungsstück nach Anspruch 7, wobei das Außenhautgewebe aufweist:
40 bis 60 Gewichtsteile einer Polypyridobisimidazol-Faser, und
40 bis 60 Gewichtsteile einer Aramidfaser.

10. Flammbeständiges Kleidungsstück nach Anspruch 7, wobei die Polypyridobisimidazol- oder Aramidfasern als Stapelfasern anwesend sind, und wobei das Polypyridimidazol-Polymer vorzugsweise Poly[2,6-dümidazo[4,5-b:4,5-e]pyridinylen-1,4-(2,5-dihydroxy)phenylen] ist.

11. Flammbeständiges Kleidungsstück nach Anspruch 7, wobei die Aramidfasern para-Aramidfasern sind, und wobei die para-Aramidfaser vorzugsweise Poly(paraphenylenterephtalamid)-Polymer aufweist.

12. Flammbeständiges Kleidungsstück nach Anspruch 7, wobei die Polypyridobisimidazol- oder Aramidfasern als Endlosfilamente anwesend sind.

13. Verfahren zur Herstellung eines flammbeständigen Kleidungsstücks mit einem inneren Thermofutter, einer Flüssigkeitssperrschicht und einem Außenhautgewebe durch Einarbeiten eines Außenhautgewebes in das Kleidungsstück, das aufweist
40 bis 60 Gewichtsteile einer Polypyridobisimidazol-Faser, und
40 bis 60 Gewichtsteile einer Aramidfaser.

14. Verfahren nach Anspruch 13, wobei die Polypyridobisimidazol-Faser Poly[2,6-diimidazo[4,5-b:4,5-e]pyridinylen-1,4-(2,5-dihydroxy)phenylen] aufweist und die Aramidfaser Poly(paraphenylen-terephthalamid) aufweist.

## Revendications

1. Vêtement résistant aux flammes ayant un tissu de revêtement extérieur comprenant:
30 à 70 parties en poids d'une fibre de polypyridobisimidazole ayant une viscosité inhérente supérieure à 20dl/g et
30 à 70 parties en poids d'une fibre d'aramide.

2. Vêtement résistant aux flammes selon la revendication 1, dans lequel la fibre de polypyridobisimidazole a une viscosité inhérente supérieure à 25dl/g, de préférence supérieure à 28dl/g.

3. Vêtement résistant aux flammes selon la revendication 1, comprenant
40 à 60 parties en poids d'une fibre de polypyridobisimidazole, et
40 à 60 parties en poids d'une fibre d'aramide.

4. Vêtement résistant aux flammes selon la revendication 1, dans lequel les fibres de polypyridobisimidazole ou d'aramide sont présentes sous la forme de fibres discontinues, et dans lequel le polypyridobisimidazole est de préférence un poly[2,6-dümidazo[4,5-b:4,5-e]-pyridinylène-1,4(2,5-dihydroxy)phénylène).

5. Vêtement résistant aux flammes selon la revendication 1, dans lequel les fibres d'aramide sont des fibres de para-aramide, et dans lequel la fibre de para-aramide comprend de préférence un polymère poly(paraphénylène téréphtalamide).

6. Vêtement résistant aux flammes selon la revendication 1, dans lequel les fibres de polypyridobisimidazole ou d'aramide sont présentes sous la forme de filaments continus.

7. Vêtement résistant aux flammes comprenant, dans l'ordre,
a) une doublure thermique interne,
b) une barrière aux liquides, et
c) un tissu de revêtement extérieur,
le tissu de revêtement extérieur comprenant:
30 à 70 parties en poids d'une fibre de polypyridobisimidazole ayant une viscosité inhérente supérieure à 20dl/g et
30 à 70 parties en poids d'une fibre d'aramide.

8. Vêtement résistant aux flammes selon la revendication 7, dans lequel la fibre de polypyridobisimidazole a une viscosité inhérente supérieure à 25dl/g, de préférence supérieure à 28dl/g.

9. Vêtement résistant aux flammes selon la revendication 7, dans lequel le tissu de revêtement extérieur comprend:
40 à 60 parties en poids d'une fibre de polypyridobisimidazole, et
40 à 60 parties en poids d'une fibre d'aramide.

10. Vêtement résistant aux flammes selon la revendication 7, dans lequel les fibres de polypyridobisimidazole ou d'aramide sont présentes sous la forme de fibres discontinues, et dans lequel le polymère polypyridimidazole est de préférence un poly[2,6-diimidazo[4,5-b:4,5-e]-pyridinylène-1,4(2,5-dihydroxy)phénylène).

11. Vêtement résistant aux flammes selon la revendication 7, dans lequel les fibres d'aramide sont des fibres de para-aramide, et dans lequel la fibre de para-aramide comprend de préférence un polymère poly(paraphénylène téréphtalamide).

12. Vêtement résistant aux flammes selon la revendication 7, dans lequel les fibres de polypyridobisimidazole ou d'aramide sont présentes sous la forme de filaments continus.

13. Procédé de fabrication d'un vêtement résistant aux flammes ayant une doublure thermique interne, une barrière aux liquides et un tissu de revêtement extérieur, en incorporant dans le vêtement un tissu de revêtement extérieur comprenant
40 à 60 parties en poids d'une fibre de polypyridobisimidazole, et
40 à 60 parties en poids d'une fibre d'aramide.

14. Procédé selon la revendication 13, dans lequel la fibre de polypyridobisimidazole comprend un poly[2,6-dümidazo[4,5-b:4,5-e]-pyridinylène-1,4(2,5-dihydroxy)phénylène) et la fibre d'aramide comprend un poly(paraphénylène téréphtalamide).
